

3,239,518

CHARGE TRANSFER COMPLEXES OF TETRAKIS-  
AMINO ETHYLENES

Hilmer E. Winberg, Wilmington, Del., assignor to E. I. du Pont de Nemours and Company, Wilmington, Del., a corporation of Delaware  
No Drawing. Filed Feb. 27, 1961, Ser. No. 91,590  
34 Claims. (Cl. 260—246)

This application is a continuation-in-part of my copending application Serial No. 836,062, filed August 26, 1959, and now abandoned.

This invention relates to, and has as its chief object provision of, novel charge transfer complexes of tetrakis(disalkylamino)ethylenes with pi or Lewis acids.

Complexes between Lewis acids and Lewis bases of widely varying structures have long been known. In many instances, one or both the acid and base components are organic, and frequently aromatic, in nature. In all but the rarest instances wherein one or both of the components is or are organic in nature the multiple linkage, from which arise the pi orbitals used in forming the complex, is part of a classically resonating multiple bond system.

This invention is generic to the charge transfer compounds or complexes of tetrakis(disalkylamino)ethylenes with Lewis acid compounds generically, i.e., with electron acceptors. The aminoethylenes are Lewis bases or electron donors. The literature shows various complexes from mixtures of Lewis acids and Lewis bases (but not involving the aminoethylenes). Many such complexes have been referred to as pi complexes. More recently, the concept that they are charge transfer complexes has become accepted—see Mulliken, J. Am. Chem. Soc. 74, 811 (1952). It is believed more nearly proper to use the generic term “charge transfer compounds” or “complexes” free of the pi connotation since, while many of these complexes owe their existence to bondings involving pi orbitals, charge transfer complexes do exist which do not involve pi orbitals. This terminology is believed proper even as applied to the diamagnetic complexes in which maximum charge transfer occurs not in the ground electronic state but in the excited state—see Orgel, Quart. Rev. Chem. Soc. 8, 422 (1954).

It has now been discovered that the tetrakis(disalkylamino)ethylenes, which are not aromatic, and, furthermore, in which the multiple carbon-carbon linkage is not part of a classically resonating multiple bond system, not only form charge transfer complexes with organic pi or Lewis acids, but also that these complexes are extremely stable and can be handled readily even at elevated temperatures. Generally the complexes with the best properties will be colored and these are preferred.

Any pi or Lewis acid can be used to form the present charge transfer complexes of the tetrakis(disalkylamino)ethylenes. Generally speaking, such Lewis acids are molecules with unfilled octets such as triphenyl boron or are unsaturated organic compounds. A preferred class are those unsaturated organic compounds containing one or more carbon-carbon multiple bonds. A particularly preferred class of such pi acids are those containing bonded to at least one of the multiply bonded carbon atoms at least one radical selected from the group consisting of nitro, nitroso, nitrile, carbacyl, trihalomethyl, 1,1-dihaloalkyl, perhaloalkyl, phenyl,  $\alpha$ -substituted-phenyl, naphthyl, sulfonyl, azo, and the like. Suitable specific examples include: dimethyl azodicarboxylate, methyl vinylsulfone,  $\alpha$ -nitro- $\beta$ -furylethylene, p-dinitrosobenzene, diethyl acetylenedicarboxylate, fumaronitrile, maleonitrile, p-diacetylbenzene and  $\alpha, \alpha, \alpha', \alpha'$ -hexachloro-p-xylene.

This present invention is generic to the addition com-

pounds of tetrakis(disalkylamino)ethylenes with unsaturated organic compounds, and preferably with organic compounds containing one or more carbon-carbon multiple bonds. Particularly preferred are the colored paramagnetic addition compounds of these tetrakis(disalkylamino)ethylenes with organic compounds containing one or more carbon-carbon multiple bonds wherein the said addition complexes or compounds are characterized as melting above 100° C. and exhibiting a spectral absorption in the range 0.5 to 4.0 microns. An especially preferred group of the colored paramagnetic addition compounds of the present invention are those compounds further characterized as containing the tetrakis(disalkylamino)ethylenes and the organic compound exhibiting pi acid character in combined molar ratios between 1:1 and 1:10. The most preferred class of these colored addition compounds of the tetrakis(disalkylamino)ethylenes with Lewis acids are those which are paramagnetic, which melt above 100° C., which are soluble to the extent of less than 0.1% in hexane, which exhibit the above spectral characteristics, wherein the said tetrakis(disalkylamino)ethylene and Lewis acid are, respectively present in mole ratios between 1:1 and 1:10 and the Lewis acid contains one or more carbon-carbon multiple bonds with at least one of the multiply bonded carbon atoms bonded to at least one radical selected from the group consisting of nitro, nitroso, nitrile, carbacyl, trihalomethyl, 1,1-dihaloalkyl, perhaloalkyl, halo, phenyl,  $\alpha$ -substituted phenyl, naphthyl, sulfonyl, azo, and the like.

The invention is generic to the colored addition compounds of tetrakis(disalkylamino)ethylenes with organic pi or Lewis acids. The alkyl substituents can be straight chain or branched chain and can vary widely in the number of carbons present therein. The structure for these aminoethylenes can be represented as follows:



wherein the  $\text{R}''_2$  which can be alike or different and taken pair-wise on each individual nitrogen or on adjacent nitrogens together joined, are used to represent alkyl and oxa and aza interrupted alkyl radicals of 1 to 10 carbons each and preferably no more than 5 carbons which can be joined pairwise as above to form 3 to 7 membered heterocycles. Suitable further illustrative examples include: tetrakis(diethylamino)ethylene, tetrakis(ethylmethylamino)ethylene, tetrakis(N-piperidino)ethylene, tetrakis(N-pyrrolidinyl)ethylene, tetrakis(morpholino)ethylene, tetrakis[N-(N'-methyl)piperazinyl]ethylene, tetrakis(dimethylaminomethyleneamino)ethylene, 1,1',3,3'-tetramethyl- $\Delta^{2,2'}$ -bi(imidazolidine), 1,1',3,3'-tetraethyl- $\Delta^{2,2'}$ -bi(imidazolidine), 1,1',3,3'-tetraethyl-1',3-dimethyl- $\Delta^{2,2'}$ -bi(imidazolidine), 1,1',3,3'-tetraethyl- $\Delta^{2,2'}$ -bi(hexahydropyrimidinone), and the like.

The following examples in which the parts given are by weight are submitted to further illustrate the invention but not to limit it.

## Example I

Under an atmosphere of nitrogen a solution of 0.344 part of tetrakis(dimethylamino)ethylene (TMAE) in 35 parts of 1,2-dimethoxyethane was added dropwise with stirring to a solution of 1.27 parts (3.0 molar proportions based on TMAE) of chloranil in 85 parts of 1,2-dimethoxyethane. A microcrystalline, dark green solid separated which was removed by filtration and subsequently air-dried. There was thus obtained 1.3 parts (81% of theory) 1/3TMAE/chloranil charge transfer compound as dark green crystals which, on heating, exhibited a color change to brown at temperatures above 150° C. Elec-

tron paramagnetic resonance analysis showed the compound to be paramagnetic, i.e., a strong EPR absorption was evidenced. The resistivity of the compound was found to be  $8.9 \times 10^8$  ohm cm. at 25° C.

*Analysis.*—Calcd. for 1/3TMAE/chloranil



C, 35.8%; H, 2.6%; N, 6.0%. Found: C, 36.2%; H, 3.1%; N, 6.8%.

A colored pattern was made by rubbing the dark green compound on the surface of a piece of paper as in writing. This pattern was easily copied in good detail using a commercial thermographic copying machine and method as described in U.S. Patents 2,740,895 and 6.

#### Example II

Under an atmosphere of nitrogen a solution of 0.86 part of TMAE in 67 parts of methylene dichloride was added dropwise with stirring over a period of 2.5 hours to a solution of 3.64 parts (an equimolar proportion based on the TMAE) of bromanil in 670 parts of methylene dichloride. A bright green solid formed which was removed by filtration, and after air-drying there was thus obtained 4.13 parts (92% of theory) of the 1/2TMAE/bromanil charge transfer compound as bright green crystals which upon being heated to 180° C. changed to a tan color and on continued heating finally decomposed at 220–230° C. The compound was paramagnetic and exhibited a strong EPR absorption. The resistivity was  $2.9 \times 10^8$  ohm cm. at 25° C.

*Analysis.*—Calcd. for 1/2TMAE/bromanil



C, 25.2%; H, 2.3%; Br, 61.0%. Found: C, 25.1%; H, 2.1%; Br, 60.8%.

The infrared spectrum, as obtained on an oil mull of the compound, exhibited maxima at 1675, 1672 (doublet), 1550, 1500, 1400, 1260, 1210, 1180, 1140, 1100, 955, 875, and 718 cm.<sup>-1</sup>. The strong bands at 1063, 1050, 870, and 700 cm.<sup>-1</sup> present in the infrared spectrum of bromanil itself are absent in the spectrum of the compound. Image patterns made with the solid compound on paper were accurately copied by the method described in Example I.

#### Example III

Under an atmosphere of nitrogen a solution of 0.172 part of TMAE in 40 parts of acetone was added dropwise with stirring to a solution of 0.526 part (one molar proportion based on the TMAE) of iodanil in 120 parts of acetone. A greenish-brown solid formed which was removed by filtration, and after air-drying there was thus obtained 0.45 part (74% of theory) of the 1/2TMAE/iodanil charge transfer compound as a greenish-brown solid which decomposed slowly on heating and was completely melted at 200° C. The solid was paramagnetic, exhibiting a strong and broad EPR absorption. The resistivity was  $1.1 \times 10^7$  ohm cm.

*Analysis.*—Calcd. for 1/2TMAE/iodanil



C, 18.5%; H, 1.7%; N, 3.9%. Found: C, 20.0%; H, 2.3%; N, 3.1%.

#### Example IV

Under an atmosphere of nitrogen a solution of 0.172 part of TMAE in 54 parts of methylene dichloride was added dropwise to a solution, with stirring, of 1.1 parts (10 molar proportions based on the TMAE) of tetracyanoethylene (TCNE) in 270 parts of methylene dichloride. The resultant brownish-black precipitate was isolated by rapid filtration and dried under reduced pressure. The brownish-black TMAE/TCNE charge transfer compound exhibited a strong EPR absorption and, therefore, was paramagnetic. The resistivity at 25° C. was  $8.9 \times 10^{11}$  ohm cm.

#### Example V

Under an atmosphere of nitrogen a solution of 0.172 part of TMAE in 67 parts of methylene dichloride was added dropwise with stirring to a solution of 0.364 part (an equimolar proportion based on the TMAE) of tetrabromo-1,2-benzoquinone in 134 parts of methylene dichloride. The resultant precipitate was isolated by filtration, and after air-drying there was thus obtained the TMAE/tetrabromo-1,2-benzoquinone charge transfer compound as a light brown solid which decomposed above 250° C. and exhibited a strong EPR absorption, i.e., was paramagnetic.

#### Example VI

Under an atmosphere of nitrogen a solution of 0.172 part of TMAE in 28 parts of benzene was added dropwise with stirring to a solution of 0.158 part (an equimolar proportion based on the TMAE) of diphenoquinone in 160 parts of benzene. The resultant precipitate was removed by filtration, and after air-drying there was thus obtained 0.25 part TMAE/diphenoquinone charge transfer compound as a light tan solid which exhibited an unusually wide EPR absorption. The resistivity of the compound was  $6.8 \times 10^{14}$  ohm cm. at 25° C.

#### Example VII

Under an atmosphere of nitrogen a solution of 0.361 part of m-dinitrobenzene in 8 parts of benzene was added dropwise with stirring to a solution of 0.43 part (an equimolar proportion based on the m-dinitrobenzene) of TMAE in 16 parts of benzene. The resulting purple solution of the TMAE/m-dinitrobenzene charge transfer compound was paramagnetic, i.e., exhibited an EPR absorption. The same preparation carried out in methylene dichloride instead of benzene afforded a red, diamagnetic solution.

#### Example VIII

Under an atmosphere of nitrogen a solution of 0.98 part of TMAE in 107 parts of methylene dichloride was added dropwise with stirring over a period of 3–4 hours to a solution of 1.36 parts (slight excess over an equimolar proportion based on the TMAE) of hexachlorocyclopentadiene in 134 parts of methylene dichloride. The solution became dark green in color, changing to a deep brown as a deep brown solid precipitated. This was removed by filtration, and after air-drying there was thus obtained 1.53 parts of the 1/1 TMAE/hexachlorocyclopentadiene charge transfer compound as a deep brown solid. The product was paramagnetic and exhibited EPR absorption.

*Analysis.*—Calcd. for a 1/1 TMAE/hexachlorocyclopentadiene compound (C<sub>15</sub>H<sub>24</sub>N<sub>4</sub>Cl<sub>6</sub>): C, 38.3%; H, 5.1%; N, 11.8%. Found: C, 38.0%; H, 5.2%; N, 11.9%.

#### Example IX

In an atmosphere of nitrogen a solution of 1.38 parts of TMAE in 107 parts of methylene dichloride was added dropwise with stirring over a period of 2 to 3 hours to a solution of one part (an equimolar proportion based on the TMAE) of dichlorofumaronitrile in 134 parts of methylene dichloride. A brownish-black precipitate formed immediately. After stirring the reaction mixture overnight, the precipitate was removed by filtration, and after air-drying there was thus obtained 2.03 parts (85% of theory) of a 1/1 TMAE/dichlorofumaronitrile charge transfer compound as a brown-black solid. The product exhibited an EPR absorption, i.e., was paramagnetic. The resistivity of the product at 25° C. was  $1.57 \times 10^{11}$  ohm cm.

#### Example X

Under an atmosphere of nitrogen a solution of 0.86 part of TMAE in 107 parts of methylene dichloride was added dropwise with stirring at room temperature to a solution of one part (a slight excess over an equimolar

proportion based on the TMAE) of p-tricyanovinyl-N,N-dimethylaniline in 268 parts of methylene dichloride. A black solid precipitate formed. The reaction mixture was stirred overnight and the solid then collected by filtration. After air-drying, there was thus obtained 0.3 part (about 16% of theory) of the 1/1 TMAE/p-tricyanovinyl-N,N-dimethylaniline charge transfer compound as a black, powdery solid. The product exhibited an EPR absorption, i.e., was paramagnetic.

*Example XI*

Under an atmosphere of nitrogen a solution of 0.344 part of TMAE in 27 parts of methylene dichloride was added dropwise with stirring to a solution of 0.276 part (an equimolar proportion based on the TMAE) of indane-1,2,3-trione in 200 parts of methylene dichloride. The resultant precipitate was isolated by filtration under nitrogen, and, after vacuum drying, the 1/2 TMAE/indane-1,2,3-trione charge transfer compound was obtained as a black, hygroscopic solid. The charge transfer compound exhibited an intense EPR absorption, i.e., was intensely paramagnetic.

*Analysis.*—Calcd. for 1/2 TMAE/indanetrione ( $C_{28}H_{32}N_4O_6$ ): N, 10.8%. Found: N, 10.8%.

*Example XII*

Under an atmosphere of nitrogen a solution of 0.172 part of TMAE in 13 parts of methylene dichloride was added dropwise with stirring to a solution of 0.27 part (an equimolar proportion based on the TMAE) of 2,4,7-trinitro-9-fluorenone in 67 parts of methylene dichloride. The resultant black precipitate was removed by filtration under nitrogen, and, after vacuum drying, there was thus obtained 0.31 part (95% of theory) of the 1/3 TMAE/2,4,7-trinitro-9-fluorenone charge transfer compound as a black, fluffy solid. The product was paramagnetic and exhibited EPR absorption.

*Analysis.*—Calcd. for 1/3 TMAE/2,4,7-trinitro-9-fluorenone ( $C_{49}H_{38}N_{13}O_{21}$ ): N, 15.9%. Found: N, 15.8%.

*Example XIII*

In a glass reactor fitted with a short packed distillation column, condensing means, and a distillation takeoff head, a mixture of 119 parts of  $\alpha,\alpha$ -dimethoxytrimethylamine and 142 parts of anhydrous pyrrolidine was heated under reflux in an oil bath at 85–106° C. Over a four-hour period 33 parts of dimethylamine was collected in a cold trap connected to the still. Methanol was then removed by distillation from the mixture as the temperature of the oil bath was slowly raised over a three-hour period to 212° C. and held at 200–212° C. for two hours. A total of 66 parts of methanol was obtained. On cooling to 90° C. the reaction residue crystallized. There was thus obtained 149.5 parts (98% of theory) of tetrakis(N-pyrrolidinyl)ethylene which after crystallization from acetonitrile was obtained as white needles melting at 91–93° C., fluorescing under ultraviolet light (3660 Å.), and chemiluminescing on exposure to air.

*Analysis.*—Calcd. for  $C_{18}H_{32}N_4$ : C, 71.0%; H, 10.6%; N, 18.4%. Found: C, 71.2%; H, 10.6%; N, 18.5%.

Under an atmosphere of nitrogen a solution of 0.30 part of tetrakis(N-pyrrolidinyl)ethylene in 17 parts of 1,2-dimethoxyethane (so-called "glyme") was added dropwise with stirring over a period of 30 minutes to a solution of 1.0 part (2.36 molar proportions based on the amine) of bromanil in 86 parts of glyme. The resulting precipitate was isolated by filtration and air-dried. There was thus obtained 0.90 part of the tetrakis(N-pyrrolidinyl)ethylene/bromanil charge transfer compound as a dark yellowish-green solid which decomposed above 207° C. and exhibited a strong EPR absorption, i.e., was paramagnetic. Image patterns made with the solid compound on paper were accurately copied by the method described in Example I.

In the same manner there was obtained from 0.76 part

of tetrakis(N-pyrrolidinyl)ethylene in 18 parts of tetrahydrofuran and 1.02 parts (two molar proportions based on the amine) of 7,7,8,8-tetracyanoquinodimethane (TCNQ) in 89 parts of tetrahydrofuran, after filtration and drying, 1.77 parts of the tetrakis(N-pyrrolidinyl)-ethylene/TCNQ charge transfer compound as a bluish-black solid decomposing above 185° C. and exhibiting a strong EPR absorption. Image patterns made with the solid charge transfer compound were easily and accurately copied by the method described in Example I.

*Example XIV*

A mixture of 59.5 parts of  $\alpha,\alpha$ -dimethoxytrimethylamine and 170 parts (2.0 molar proportions based on the amine) of anhydrous piperidine in a glass reactor was attached to a still as in Example XIII and was heated at the reflux in an oil bath until evolution of dimethylamine ceased. Methanol was then distilled from the reaction mixture as the temperature of the heating bath was slowly raised over a period of eight hours to 140° C. A total of 31.6 parts (theory, 32 parts) of methanol was obtained. Removal of all material (including excess piperidine) volatile below a bath temperature of 170° C., while maintaining the reactor at a pressure corresponding to 0.55 mm. of mercury, afforded 80 parts (89% of theory) of tetrakis(piperidino)ethylene as a residue which crystallized on cooling. After recrystallization from acetonitrile, the product melted at 59–61° C.

*Analysis.*—Calcd. for  $C_{22}H_{40}N_4$ : C, 73.3%; H, 11.2%; N, 15.5%. Found: C, 72.8%; H, 11.9%; N, 15.5%.

Under an atmosphere of nitrogen a solution of 0.90 part of tetrakis(N-piperidino)ethylene in 17 parts of glyme was added dropwise with stirring to a solution of 1.02 parts (two molar proportions based on the amine) of TCNQ in 178 parts of warm glyme. The resulting precipitate was isolated by filtration and air-dried. There was thus obtained 0.04 part of the tetrakis(N-piperidino)ethylene/TCNQ charge transfer compound as a blue-black solid which decomposed at 243° C. and exhibited both a strong EPR absorption, i.e., was paramagnetic, and a wide spectral absorption band with a peak at 3.0 $\mu$ . Image patterns made with the solid compound on paper were accurately copied by the method described in Example I.

In the same manner there was obtained from 0.36 part of tetrakis(N-piperidino)ethylene in 17 parts of glyme and 0.184 part (one molar proportion based on the ethylene) of diphenoxquinone in 65 parts of glyme, after filtration and drying, 0.05 part of the tetrakis(N-piperidino)ethylene/diphenoxquinone charge-transfer compound as a brown solid decomposing above 180° C. and exhibiting a strong EPR absorption. Image patterns made with the solid charge transfer compound were easily and accurately copied by the method described in Example I.

*Example XV*

A mixture of 26.8 parts of  $\alpha,\alpha$ -dimethoxytrimethylamine and 41.2 parts of anhydrous morpholine was heated in a glass reactor attached to a still as in Example XIII at the reflux in an oil bath at 98–110° C. After 2.5 hours under these conditions, dimethylamine evolution ceased. Methanol was then distilled from the reaction mixture as the temperature of the bath was slowly raised over a period of four hours to 200° C. and held at that temperature for an additional 0.5 hour. Continued distillation under reduced pressure afforded 20.4 parts (42% of theory) of bis(morpholino)methoxymethane as a clear, colorless liquid boiling at 103–108° C. under a pressure corresponding to 1.0–1.2 mm. of mercury. On cooling, the product crystallized and melted at 64–67.5° C. after recrystallization from methylcyclohexane.

*Analysis.*—Calcd. for  $C_{10}H_{20}N_2O_3$ : C, 55.5%; H, 9.3%; N, 13.0%. Found: C, 55.7%; H, 9.2%; N, 13.2%.

On cooling, the still residue from the isolation of the above bis(morpholino)methoxymethane solidified. There

was thus obtained 21.8 parts (41% of theory) of tetrakis(morpholino)ethylene. After recrystallization from ethyl acetate, the product melted at 170-171° C.

*Analysis.*—Calcd. for  $C_{12}H_{32}N_4O_4$ : N, 15.2%. Found, N, 15.4%.

Under an atmosphere of nitrogen a solution of 0.92 part of tetrakis(morpholino)ethylene in 18 parts of tetrahydrofuran was added dropwise to 1.02 parts (two molar proportions based on the ethylene) of TCNQ in 89 parts of warm tetrahydrofuran. The resulting precipitate was isolated by filtration and air-dried. There was thus obtained 0.73 part of the tetrakis(morpholino)ethylene/TCNQ charge transfer compound as a blue-black solid which decomposed above 213° C. and exhibited both a strong EPR absorption, i.e., was paramagnetic, and a wide spectral absorption band with a peak at 3.0 $\mu$ . Dilute solutions in tetrahydrofuran or acetone were green in color. Image patterns made with the solid compound on paper were accurately copied by the method described in Example I.

#### Example XVI

As in Example XIII, a mixture of 11.9 parts of  $\alpha,\alpha$ -dimethoxytrimethylamine and 20.0 parts of N-methylpiperazine was heated at 130-210° C. until evolution of dimethylamine and methanol had ceased. Continued distillation of the reaction mixture under reduced pressure afforded 7.8 parts (32% of theory) of bis[N-(N'-methyl)piperazinyl]methoxymethane as a clear, colorless liquid boiling at 106-110° C. under a pressure corresponding to 0.9 mm. of mercury.

*Analysis.*—Calcd. for  $C_{12}H_{26}N_4O$ : C, 59.5%; H, 10.8%. Found: C, 59.9%; H, 10.8%.

On cooling, the still residue from the isolation of the above substituted methoxymethane crystallized. There was thus obtained 11.1 parts (53% of theory) of tetrakis[N-(N'-methyl)piperazinyl]ethylene which after recrystallization from acetonitrile melted at 79.0-80.5° C.

*Analysis.*—Calcd. for  $C_{22}H_{44}N_8$ : N, 26.6%. Found: N, 26.6%.

Under an atmosphere of nitrogen a solution of 1.05 parts of tetrakis[N-(N'-methyl)piperazinyl]ethylene in 18 parts of tetrahydrofuran was added dropwise to 1.02 parts (two molar proportions based on the ethylene) of TCNQ in 89 parts of warm tetrahydrofuran. The resulting precipitate was isolated by filtration and air-dried. There was thus obtained 0.42 part of the tetrakis[N-(N'-methyl)piperazinyl]ethylene/TCNQ charge transfer compound as an acetone-soluble, fluffy black solid which decomposed above 218° C. and exhibited both a strong EPR absorption, i.e., was paramagnetic, and a wide spectral absorption band with a peak at 3.0 $\mu$ . Dilute solutions in tetrahydrofuran and acetone were green in color. Image patterns made with the solid compound on paper were accurately copied by the method described in Example I.

In the same manner there was obtained from 0.84 part of tetrakis[N-(N'-methyl)piperazinyl]ethylene in 17 parts of glyme and 0.98 part (two molar proportions based on the ethylene) of tetrachloro-o-quinone, after filtration and drying, the tetrakis[N-(N'-methyl)piperazinyl]ethylene/tetrachloro-o-quinone charge transfer compound as a tan-colored solid which rapidly became tacky in air. It exhibited a strong EPR absorption, i.e., was paramagnetic. Image patterns made with the solid compound on paper were accurately copied by the method described in Example I.

#### Example XVII

As in Example XIII, a mixture of 29.8 parts of  $\alpha,\alpha$ -dimethoxytrimethylamine and 23.3 parts of N,N'-dimethyl-ethylenediamine was heated in an oil bath at 100-156° C. until evolution of dimethylamine and methanol had ceased. Continued distillation of the reaction residue afforded 20.4 parts (83% of theory) of 1,1',3,3'-tetramethyl- $\Delta^{2,2'}$ -bi(imidazolidine) as a clear, colorless

liquid which boiled at 96-97° C. under a pressure corresponding to 8 mm. of mercury and which crystallized on cooling to a low-melting solid. This bicyclic tetrakis(disubstitutedamino)ethylene chemiluminesces strongly in air with evolution of heat. Solutions of the product in cyclohexane also chemiluminesce strongly in the presence of air.

*Analysis.*—Calcd. for  $C_{10}H_{20}N_4$ : C, 61.2%; H, 10.3%. Found: C, 61.2%; H, 10.5%.

Under an atmosphere of nitrogen a solution of 0.98 part of 1,1',3,3'-tetramethyl- $\Delta^{2,2'}$ -bi(imidazolidine) in 18 parts of tetrahydrofuran was added dropwise to 2.04 parts (two molar proportions based on the amine) of TCNQ in 155 parts of warm tetrahydrofuran. The resulting precipitate was isolated by filtration and air-dried. There was thus obtained 2.9 parts of the 1,1',3,3'-tetramethyl- $\Delta^{2,2'}$ -bi(imidazolidine)/TCNQ charge transfer compound as an acetone-soluble, deep blue solid which decomposed above 220° C. and exhibited a strong EPR absorption, i.e., was paramagnetic. Image patterns made with the solid compound on paper were accurately copied by the method described in Example I.

#### Example XVIII

As in Example XIII, a mixture of 87 parts of  $\alpha,\alpha$ -dimethoxytrimethylamine and 85 parts of N,N'-diethyl-ethylenediamine was heated under reflux in an oil bath at 85-105° C. until evolution of dimethylamine became slow. Methanol was then distilled from the reaction mixture as the bath temperature was slowly raised until a final temperature of 200° C. was reached. Continued distillation of the reaction mixture under reduced pressure afforded 69.5 parts (76% of theory) of 1,1',3,3'-tetraethyl- $\Delta^{2,2'}$ -bi(imidazolidine) as a light yellow liquid boiling at 79-82° C. under a pressure corresponding to 0.5 mm. of mercury. The product chemiluminesced strongly on exposure to air.

*Analysis.*—Calcd. for  $C_{14}H_{28}N_4$ : C, 66.6%; H, 11.2%; N, 22.2%. Found: C, 66.9%; H, 11.3%; N, 21.9%.

Under an atmosphere of nitrogen a solution of 0.475 part of 1,1',3,3'-tetraethyl- $\Delta^{2,2'}$ -bi(imidazolidine) in 17 parts of glyme was added dropwise with stirring over a period of 30 minutes to a solution of 1.46 parts (3.1 molar proportions based on the amine) of chloranil in 86 parts of glyme. The resulting precipitate was isolated by filtration and air-dried. There was thus obtained 1.55 parts of the 1,1',3,3'-tetraethyl- $\Delta^{2,2'}$ -bi(imidazolidine)/chloranil charge transfer compound as a bright green solid which decomposed above 140° C. and exhibited a strong EPR absorption, i.e., was paramagnetic. Image pattern made with the solid compound on paper were accurately copied by the method described in Example I.

In the same manner there was obtained from 0.95 part of 1,1',3,3'-tetraethyl- $\Delta^{2,2'}$ -bi(imidazolidine) in 18 parts of tetrahydrofuran and 1.53 parts (two molar proportions based on the amine) of TCNQ in 133 parts of tetrahydrofuran, after filtration and drying, 2.71 parts of the 1,1',3,3'-tetraethyl- $\Delta^{2,2'}$ -bi(imidazolidine)/TCNQ charge transfer compound as a dark blue solid decomposing above 170° C. and exhibiting a strong EPR absorption. Image patterns made with the solid compound were easily and accurately copied by the method described in Example I.

In the same manner there was obtained from 0.24 part of 1,1',3,3'-tetraethyl- $\Delta^{2,2'}$ -bi(imidazolidine) in 17 parts of glyme and 0.87 part (two molar proportions based on the amine) of tetra(p-nitrophenyl)ethylene in 86 parts of glyme, after filtration and air-drying, the 1,1',3,3'-tetraethyl- $\Delta^{2,2'}$ -bi(imidazolidine)/tetra(p-nitrophenyl)ethylene charge transfer compound as a reddish-brown solid which exhibited a strong EPR absorption, i.e., was paramagnetic.

#### Example XIX

A mixture of 23.8 parts of  $\alpha,\alpha$ -dimethoxytrimethylamine and 20.4 parts of N-ethyl-N'-methylethylenedi-

amine was heated as in Example XIII to a bath temperature of 160° C. over a period of six hours, with the dimethylamine and methanol evolved in the reaction being removed by distillation. Essentially the theoretical quantity of the latter was obtained. Continued distillation of the reaction residue under reduced pressure afforded 17.2 parts (77% of theory) of 1,3'-diethyl-1',3-dimethyl- $\Delta^{2,2'}$ -bi(imidazolidine) as a light yellow liquid boiling at 80-82° C. under a pressure corresponding to 0.25 mm. of mercury. The product chemiluminesced strongly on exposure to air.

*Analysis.*—Calcd. for C<sub>12</sub>H<sub>24</sub>N<sub>4</sub>: C, 64.2%; H, 10.8%; N, 25.0%. Found: C, 64.2%; H, 11.0%; N, 24.4%.

Under an atmosphere of nitrogen a solution of 0.48 part of 1,3'-diethyl-1',3-dimethyl- $\Delta^{2,2'}$ -bi(imidazolidine) in 17 parts of glyme was added dropwise with stirring to a solution of 1.36 parts (two molar proportions based on the amine) of 2,4,7-trinitro-9-fluorenone in 65 parts of glyme. The resulting precipitate was isolated by filtration and air-dried. There was thus obtained 1.0 part of the 1,3'-diethyl-1',3-dimethyl- $\Delta^{2,2'}$ -bi(imidazolidine)/2,4,7-trinitro-9-fluorenone charge transfer compound as an acetone-soluble, purple-black, fluffy solid which exhibited a strong EPR absorption, i.e., was paramagnetic. Image patterns made with the solid compound on paper were accurately copied by the method described in Example I.

#### Example XX

A mixture of 73.4 parts of  $\alpha,\alpha$ -dimethoxytrimethylamine, 62.6 parts of N,N'-dimethyl-1,3-propanediamine, and 132 parts of benzene was heated at the reflux with the benzene/methanol azeotrope, boiling at 58° C. at atmospheric pressure, being removed continuously as it was formed. The dimethylamine formed concurrently was vented to the atmosphere. Heating was continued until the azeotrope no longer distilled over and the benzene was then removed by evaporative distillation. Continued distillation of the residue under reduced pressure afforded 20.8 parts (24% of theory) of 1,3-dimethyl-2-methoxyhexahdropyrimidine as a colorless liquid boiling at 62-66° C. under a pressure corresponding to 25 mm. of mercury.

*Analysis.*—Calcd. for C<sub>7</sub>H<sub>16</sub>N<sub>2</sub>O: C, 58.3%; H, 11.2%; N, 19.4%. Found: C, 58.6%; H, 11.2%; N, 19.4%.

Continued distillation of the reaction residue after removal of the 1,3-dimethyl-2-methoxyhexahdropyrimidine afforded 23.3 parts (34% of theory) of 1,1',3,3'-tetramethyl- $\Delta^{2,2'}$ -bi(hexahdropyrimidine) as a light yellow liquid boiling at 104-105° C. under a pressure corresponding to 8.5 mm. of mercury. The product luminesced strongly on exposure to air.

*Analysis.*—Calcd. for C<sub>12</sub>H<sub>24</sub>N<sub>4</sub>: N, 25.0%. Found: N, 25.1%.

Under an atmosphere of nitrogen a solution of 0.23 part of 1,1',3,3'-tetramethyl- $\Delta^{2,2'}$ -bi(hexahdropyrimidine) in 18 parts of tetrahydrafuran was added dropwise with stirring to a solution of 1.27 parts (three molar proportions based on the amine) of bromanil in 89 parts of tetrahydrafuran. The resulting precipitate was isolated by filtration and air-dried. There was thus obtained the 1,1',3,3'-tetramethyl- $\Delta^{2,2'}$ -bi(hexahdropyrimidine)/bromanil charge transfer compound as a greenish-tan solid which decomposed above 150° C. and exhibited a strong EPR absorption, i.e., was paramagnetic. Image patterns made with the solid compound on paper were accurately copied by the method described in Example I.

In a similar manner there was obtained from 0.56 part of 1,1',3,3'-tetramethyl- $\Delta^{2,2'}$ -bi(hexahdropyrimidine) in 18 parts of tetrahydrafuran and 1.02 parts (two molar proportions based on the amine) of TCNQ in 89 parts of warm tetrahydrafuran, after filtration and drying, the 1,1',3,3'-tetramethyl- $\Delta^{2,2'}$ -bi(hexahdropyrimidine)/TCNQ charge transfer compound as a blue-black solid

which decomposed above 235° C. Dilute acetone solutions were bright green colored. It exhibited both a strong EPR absorption, i.e., was paramagnetic, and a wide spectral absorption band with a peak at 3.0 $\mu$ . Image patterns made with the solid compound on paper were accurately copied by the method described in Example I.

As stated above, the charge transfer compounds of the tetrakis(dialkylamino)ethylenes can be formed with any Lewis acid. In addition to the fully detailed examples just given, charge transfer compounds can be prepared from many other Lewis acids, of which wide numbers are known. For instance, when methylene dichloride solutions of TMAE and maleic anhydride were mixed, the mixture turned red immediately with evolution of heat and apparent further reaction. When methylene dichloride solutions of TMAE and tetrachlorobenzoquinone were mixed, a blue-green precipitate formed which exhibited an intense EPR absorbance. The supernatant blue solution and the blue-green precipitate exhibited separately no EPR absorption after about two hours. Presumably subsequent reaction of the charge transfer compound occurred. When methylene dichloride solutions of TMAE and TCNE were mixed in a different ratio than given in Example IV, a clear red solution was obtained which exhibited an intense EPR absorbance which persisted, apparently undiminished, for 72 hours. The colored charge transfer compound was thus strongly paramagnetic. When methylene dichloride solutions of TMAE and indanetrione, i.e., triketohydrindene, were mixed, the mixture turned red immediately and a dark precipitate subsequently formed. The solid was intensely paramagnetic.

When TMAE and acrylonitrile were mixed, a red-colored solution resulted which exhibited an EPR absorbance. When TMAE and tetrachloroethylene were mixed, the mixture turned yellow, but no EPR absorbance was exhibited. Similar results were obtained with TMAE and styrene. In these two latter instances, the charge transfer compounds formed were presumably diamagnetic in the ground state. Solutions of TMAE and hexachloro-1,3,5-cyclohexanetrione formed a red-orange precipitate with concomitant evolution of heat. The solid exhibited an EPR absorbance. When alcohol solutions of TMAE and riboflavin were mixed, a brilliant red-colored solution resulted which gave an intense EPR signal.

The present invention is generic to the charge transfer complexes between the tetrakis(dialkylamino)ethylenes and pi or Lewis acids broadly. The pi acids involved will normally have at least one carbon atom multiply bonded to another atom, generally another carbon atom or an oxygen, nitrogen, or sulfur atom. A particularly useful class of the pi acids are those wherein at least one carbon is multiply bonded to another carbon, such as in an ethylenic group or in a benzene or other carbocyclic or heterocyclic aromatic nucleus. Especially outstanding amongst these pi acids, wherein at least one carbon is multiply linked to another carbon, are those compounds wherein at least one of the carbons involved in the multiple linkage carries at least one electronegative substituent. These electronegative substituents are recognized and described as such in the literature and are frequently also referred to as substituents which, when present on ring carbon of an aromatic nucleus, tend to direct any entering substituent radical into the meta-position, i.e., the so-called meta-orienting groups. These substituents have also been described by Price, Chem. Rev. 29, 58 (1941), in terms of the electrostatic polarizing force measured in dynes of the said substituent groups on an adjacent double bond of a benzene nucleus. Quantitatively, any substituent which has or exhibits an electrostatic polarizing force in dynes greater than 0.50 is classed as electronegative and meta-orienting. These substituents include nitroalkyl, such as 2-nitropropyl, nitromethyl; polyhaloalkyl, such as di-

chloro-methyl, trichloromethyl, trifluoromethyl; nitroso and nitro; ammonium and quaternary ammonium and ammonium alkyl and quaternary ammonium alkyl, such as ammonium, methyl quaternary trimethylammonium, ammonium, and quaternary trimethylammonium methyl; carbamoyl and substituted carbamoyl; carbacyl, such as acetyl and formyl; polycyanoalkyl, such as dicyanomethyl; hydrocarboylloxycarbonyl, such as methoxy-carbonyl, and other carbacyl esters; carboxyl and sulfo and other acyl groups; hydrocarbyl sulfonyl, such as methylsulfonyl, and other sulfonic acid esters; formyl, acetyl, propionyl, and other carbacyl groups; and nitrile.

In accordance with the present invention, it has been found that reaction of any tetrakis(dialkylamino)ethylene with any pi or Lewis acid produces charge transfer compounds which are characteristically colored. The reaction takes place upon merely mixing the reactants alone or in an inert solvent or solvents. Any convenient temperature can be used, but low temperatures sometimes are desirable to avoid or suppress other reactions. In those instances wherein the pi acid is a solid, the charge transfer compound can be made by simply mixing the solid with the liquid or solid tetrakis(dialkylamino)ethylene and suitably mixing. If desired, the reaction mixture can be heated slightly. In those instances wherein the pi acid is a liquid, the liquid can be mixed with the liquid or solid tetrakis(dimethylamino)ethylene. In those instances where the pi acid is solid but exhibits an appreciable vapor pressure either under slightly elevated temperature or under greatly reduced pressure, the vapors from the solid pi acid and the liquid or solid tetrakis(dialkylamino)ethylene can be brought together in a suitable reaction zone and the complex formed thereby. Solvents or diluents for preparation include: ethers, acetone, methylene chloride, chloroform, benzene, hexane, cyclohexane, acetonitrile, carbon tetrachloride, toluene, dimethylformamide, dimethylsulfoxide, 1,2-dimethoxyethane, pyridine, picolines, and the like. Diluents in which the complex is insoluble are advantageous since the complex tends to be protected from further attack by excess Lewis acid or base. The charge transfer complexes can be purified by a variety of procedures depending on the stability and solubility of the individual complexes. These include solution and precipitation from suitable solvents, sublimation, and zone refining.

The tetrakis(dialkylamino)ethylene charge transfer compounds with the stronger pi acids are paramagnetic and thus have usefulness in recognized applications for paramagnetic materials. These paramagnetic complexes are generically characterized by exhibiting paramagnetic absorption in the electron paramagnetic resonance spectrum (EPR absorption).

A still further use of the tetrakis(dialkylamino)ethylene charge transfer compounds which are paramagnetic resides in an additional characteristic physical property of such complexes. Thus, these paramagnetic tetrakis(dialkylamino)ethylene compounds exhibit strong, broad absorption in the near infrared region, e.g., from 0.5 to 2.0 microns, generally centered around 1.0 micron. Based on this property, such complexes find significant use as the coloring agent, or pigment, in writing inks which will permit reproduction of text matter by thermographic processes.

Thermographic copying represents a convenient and easy method of rapidly copying text material dry. However, operability of the process requires that the text material to be copied must absorb in the infrared. Otherwise there is no heat buildup and accordingly no copy is formed on the thermographic paper. Printed material, wherein the text matter is in pigmented inks, is satisfactory since the pigment materials for these inks do absorb in the infrared. The same is true of typewritten matter, whether it be the original copy or carbon copies thereof, since again the text matter is defined by carbon particles which absorb in the infrared. However, most

fountain pen inks, and in particular ballpoint inks, achieve their characteristic color through the use of dyes or pigments which do not absorb in the infrared but only in the visible. Accordingly, text matter appearing in these types of inks cannot be copied by a thermographic process. The paramagnetic tetrakis(dialkylamino)ethylene charge transfer complexes in absorbing in the near infrared permit direct, ready, and easy thermographic copying of lettertext matter defined by inks carrying these complexes as the coloring, or pigmenting, agent.

All the tetrakis(dialkylamino)ethylene charge transfer pi complexes, including both the diamagnetic and paramagnetic types, are generically colored and accordingly find use in any of the many well-known and established uses for colored materials. Thus, in the case of colored solutions, obtainable with quite weak pi acids, e.g., nitrobenzene, these are useful in obtaining decorative color effects. In the case of the tetrakis(dialkylamino)ethylene charge transfer pi complexes with stronger pi acids, the complexes are colored solids irrespective of whether the complex is paramagnetic or not. These colored solid complexes find use in any of the many well-established fields, such as dyes, pigments, for both paints and plastics, and colored fillers for the latter.

Since all the tetrakis(dialkylamino)ethylene charge transfer complexes are colored, the controlled formation thereof forms the basis for still another use, viz., the reproduction of text matter by impact printing, i.e., by the pressure formation of graphic images. Thus, one sheet of a carrier, e.g., paper, is impregnated with a solution of tetrakis(dialkylamino)ethylene and the solvent removed via evaporation, leaving the tetrakis(dialkylamino)ethylene deposited in, on, and through the paper carrier. Another separate sheet of paper is similarly so treated with a pi acid. A laminate of the two sheets will reproduce a colored image in the second sheet made by pressure on the first sheet.

As stated and illustrated in the foregoing, this invention is generic to the charge transfer compounds of the tetrakis(dialkylamino)ethylenes and Lewis acids broadly. The "tetrakis(dialkylamino)ethylenes" is intended to include those compounds not only where there are two discrete, i.e., separate, substituents aliphatic in character (i.e., aliphatic and cycloaliphatic) on each amino nitrogen but also those wherein two substituents on individual or adjacent nitrogens are embodied in a single divalent radical, making with the amino nitrogen a monoaza, diaza, and/or oxa/aza heterocycle of from three to seven total ring members wherein any substituents on ring members are solely saturated hydrocarbon of no more than eight carbons each. Thus, the said term describes not only the simple tetrakis(dialkylamino)ethylenes but also the more complicated structures wherein substituents on individual or adjacent amino nitrogen are together joined pairwise, either directly or through intervening heterocyclic oxa or aza members. The first member of this large class of tetrakis(dialkylamino)ethylenes, i.e., TMAE, is an extremely reactive and peculiar compound which can be prepared in excellent yield by the direct interaction between chlorotrifluoroethylene and dimethylamine in the manner of Prueett et al., J. Am. Chem. Soc. 72, 3646 (1950). None of the rest of the class of the tetrakis(dialkylamino)ethylenes, even including the first next adjacent methylene homolog, i.e., tetrakis(diethylamino)ethylene, can be made by this same technique substituting the requisite different secondary amine.

The other tetrakis(dialkylamino)ethylenes needed as intermediates for preparing the charge transfer compounds of the present invention are new compounds and can be prepared by the interaction between the requisite secondary amine and the hydrocarbon amide acetals, which may also be described as disubstituted aminodihydrocarboylmethanes, preferably those of relatively short chain length, in the manner disclosed and claimed in the application of Winberg, Serial No. 91,589, filed

concurrently herewith and now abandoned but refiled as the continuation-in-part application Serial No. 174,404, on February 20, 1962. This interaction between the requisite secondary amine and amide acetal intermediates, i.e., the disubstituted amino-1,1-dihydrocarbyloxy-methanes, is basically a substitution or substitution/condensation reaction in which the entering secondary amine moiety is substituted for the disubstituted amino moiety of the amide acetal and also for one of the hydrocarbyloxy moieties of the amide acetal and with ultimate splitting out of another molecule of the hydroxyhydrocarbyl compound and resultant dimerization to the formation of the desired tetrakis(dialkylamino)ethylene, all in accord with the following stoichiometry:



wherein the R's, which can be alike or different, are monovalent alkyl or cycloalkyl radicals, generally of no more than eight carbons each, which can be together joined to form with the intervening nitrogen a heterocycle of from three to seven ring members; the R's which can also be alike or different, or together joined, are monovalent alkyl, aryl, aralkyl, alkaryl, or cycloalkyl radicals and, when together joined, form with the two oxygens and intervening carbon a 1,3-dioxaheterocycle of from five to seven ring members; and the R''s, which can also be alike or different or together joined pairwise on the same or different nitrogens, are monovalent alkyl or cycloalkyl hydrocarbon or oxa- and/or azahydrocarbon radicals of no more than eight carbons each. In any event, when the two R''s are together joined, they form with the indicated amine nitrogen a monoazacarbocycle, an oxazacarbocycle, or a diazacarbocycle of from three to seven ring members.

Because of easier conversion to the desired tetrakis(dialkylamino)ethylenes, the short chain hydrocarbon amide acetals are preferred wherein the radicals pendent on the nitrogen and the two oxy oxygens are short chain, saturated hydrocarbon, and oxa- and azahydrocarbon radicals of no more than six chain or ring members each. Ideally speaking, the best amide acetal intermediate is the one where all such radicals are the shortest, viz., 1,1-dimethoxydimethylamine, i.e., the dimethyl acetal of N,N-dimethylformamide. The reaction is effected simply by mixing the two coreactants, generally with the secondary amine in excess, and heating to drive off the hydroxyhydrocarbyl compound, i.e., alcohol or phenol, and amine formed in accord with the foregoing stoichiometry.

Thus, the resulting substituted secondary amine corresponding to the secondary amino moiety of the amide acetal coreactant will be removed by distillation as the reaction proceeds, as will any resulting alcohol or phenol, through the condensation/substitution of the second disubstituted amino fragment from the entering secondary amine for one of the hydrocarbyloxy fragments of the amide acetal. The final dimerization step is effected substantially solely thermally, and in order to insure maximum yield of the desired tetrakis(dialkylamino)ethylenes, the reaction will finally be carried out in the temperature range 125-250° C., except in those instances where short-chain diamines are the entering secondary amines, resulting in the formation of cyclic tetrakis-substituted aminoethylenes, in which instance reaction temperatures need not normally be carried much above the 80-125° C. range.

The reaction is an easy one to carry out, requiring only that the necessary two coreactants be brought together and heated. To avoid possible side reactions and

other complicating factors, the reaction is normally carried out in a dry, inert atmosphere, e.g., dry N<sub>2</sub>. The substituted secondary amine corresponding to the disubstituted amino moiety of the starting amide acetal coreactant will normally be removed by simple distillation. Ideally speaking, this disubstituted amine will be sufficiently low boiling that it can be permitted to vent as a gas through the reflux condenser of the distillation head normally used. The alcohol or phenol resulting from the condensation reaction between a second molar proportion of the entering secondary amine and one of the hydrocarbyloxy moieties of the amide acetal coreactant will normally be condensed and removed as a liquid distillate as formed.

While no reaction solvent at all is required, for ease and convenience it may sometimes be desirable to use an inert hydrocarbon or hydrocarbon ether solvent in excess to assure good contact between the two coreactants. Since many of the lower alcohols form azeotropes with various of the hydrocarbon solvents, it frequently develops that the alcohol/hydrocarbon solvent azeotrope simply is distilled from the reaction mixture, and when azeotrope formation ceases, the reaction for the formation of the bis(disubstitutedamino)hydrocarbyloxymethane is substantially complete. Under such conditions, i.e., using an inert solvent, the reaction mixture normally will not reach the temperatures necessary for the formation of the tetrakis(disubstitutedamino)ethylenes except, as mentioned before, for the diamines and resultant cyclic aminoethylenes. For the tetrasubstituted products, either no reaction diluent is used and the reaction is driven to completion solely thermally, or for convenience, an inert reaction solvent is used and the reaction driven to completion therewith to the formation of the bis(disubstitutedamino)hydrocarbyloxymethane. The reaction diluent will then be removed by distillation and the tetrakis(disubstitutedamino)ethylene formed by further heating of the bis(disubstitutedamino)hydrocarbyloxymethane.

The requisite amide acetal intermediates can be prepared by the method of Meerwein, Angew. Chem. 71,530 (1959), by reaction between a hydrocarbon ether, a hydrocarbyl fluoride, and silver fluoborate to form a trihydrocarbyloxonium fluoborate which is then reacted with the requisite N,N-dihydrocarbyl-substituted carboxamide to form the intermediate oxonium fluoborate derivative of the amide, i.e., an  $\alpha$ -(N,N-dihydrocarbylamino)- $\alpha$ -(hydrocarbyloxy)hydrocarbonium fluoborate, which is subsequently further reacted with an alkali metal alcoholate to form the desired amide acetal and, as a co-product, the alkali metal fluoborate. Also, as disclosed in the same reference, the intermediate higher amide acetals can be prepared by alcohol exchange with the lower amide acetals in accord with the following stoichiometry:



where R'' is of greater carbon content than R'.

In view of the innate complexity of the silver fluoborate synthesis, the latter, i.e., the alcohol exchange route, will, for reasons of convenience, generally be preferred. Thus, the silver fluoborate synthesis will normally be used to prepare the first member of the series, i.e., the dimethyl acetal of N,N-dimethylformamide, which will then be used in alcohol exchange to prepare any desired higher hydrocarbyloxy amide acetals. The same generally applies to any desired higher hydrocarbylamino amide acetals in which an amine exchange reaction in accord with the following stoichiometry will serve to prepare any desired higher hydrocarbylamino amide acetals:



where R'' is of greater carbon content than R.

In both these alcohol and amine exchange reactions, the cyclic products can also be obtained, i.e., by the use of a glycol to obtain the cyclic hydrocarbyloxy moiety or by use of a cyclic secondary amine to obtain the cyclic amino moiety of the amide acetals.

The preferred method of preparing the necessary intermediate amide acetals involves the reaction of an alkali metal of alkaline earth metal salt of the desired alcohol or phenol with the requisite  $\alpha,\alpha$ -dihalosubstituted tertiary amine in accord with the following stoichiometry:



wherein the R's, which can be alike or different, are monovalent alkyl or cycloalkyl radicals of no more than 8 carbons each, which can be together joined to form a saturated monoaza, diaza, or oxaza heterocycle of 3-7 ring members; the X's, which can be alike or different, are halogens of atomic No. from 9-35; M is an alkali metal or an alkaline earth metal; R' is a monovalent alkyl, aryl, aralkyl, alkaryl, or cycloalkyl radical of no more than 8 carbons; and m and n are integers from 1-2, inclusive, depending on the valence of the metal M and such that  $m+n=3$ . When n is 2, the R' radicals can be together joined to form with the intervening carbon and two oxygens a 1,3-dioxacarbocycle of 5 to 7 ring members. This preferred synthesis of the intermediates forms the subject matter of Brown U.S. Patent 3,092,637.

In addition to the aforesaid new tetrakis(disubstituted-amino)ethylenes and the necessary amide acetal and secondary amine coreactants given in the foregoing detailed examples, other such coreactants of these same generic types can be so similarly used to give still further amino ethylene intermediates for the charge transfer compounds of the present broad product invention. Thus, there can be used such other formamide acetals as N-(dimethoxy-methyl)-N-methyl-n-octylamine, N-diethoxymethylisobutylamine, N-diethoxymethyl-N-ethyl-p-toluidine, N-diethoxymethylpyrrolidine, N-diisopropoxymethylmorpholine, and the like. In preparing the new tetrakis(disubstituted-amino)ethylenes there can be used such cyclic secondary amines as ethyleneimine, i.e., aziridine, azetidine, i.e., azacyclobutane, perhydroazepine,  $\Delta^3$ -pyrrolidine, i.e., 2,5 dihydroazoline, 1,2,2-trimethylhydrazine, and the like. Reaction of these additional amine species with the dimethyl acetal of N-dimethylformamide results, respectively, in the formation of the following tetrakis(cyclic and acyclic disubstitutedamino)ethylenes: 1,1,2,2-tetrakis (1-aziridinyl)ethylene, 1,1,2,2-tetrakis(1-azetidinyl)ethylene, 1,1,2,2 - tetrakis(1 - hexahydroazepinyl)ethylene, 1,1,2,2 - tetrakis(1,2,5 - dihydroazolinyl)ethylene, i.e., 1,1,2,2-tetrakis(1- $\Delta^3$ -pyrrolinyl)ethylene, 1,1,2,2-tetrakis [1-(1,2,2-trimethylhydrazinyl)]ethylene, and the like.

Since obvious modifications and equivalents in the invention will be evident to those skilled in the chemical arts, I propose to be bound solely by the appended claims.

The embodiments of the invention in which an exclusive property or privilege is claimed are defined as follows:

1. A charge transfer complex of (1) an amino compound of the formula



wherein the R''s are selected from the group consisting, individually, of monovalent alkyl and cycloalkyl hydrocarbon of up to 10 carbons, jointly on each nitrogen, of divalent alkylene, cycloalkylene and oxa- and azahydrocarbon of up to 10 carbons and forming a heterocyclic structure of 3-7 ring members, and, jointly on adjacent nitrogens, of divalent alkylene, cycloalkylene and oxa- and azahydrocarbon of up to 10 carbons and forming a heterocyclic structure of 3-7 ring members and (2) an organic Lewis acid containing at least one multiple bond between carbon and a member of the group consisting

of carbon, nitrogen, oxygen and sulfur, the mole ratio of (1) to (2) being between 1:1 and 1:10.

2. The complex of claim 1 wherein the amino compound is tetrakis(dimethylamino)ethylene.
3. A charge transfer complex of an amino compound of claim 1 and chloranil.
4. A charge transfer complex of an amino compound of claim 1 and bromanil.
5. A charge transfer complex of an amino compound of claim 1 and iodanil.
6. A charge transfer complex of an amino compound of claim 1 and tetracyanoethylene.
7. A charge transfer complex of an amino compound of claim 1 and tetrabromo-1,2-benzoquinone.
8. A charge transfer complex of an amino compound of claim 1 and diphenoquinone.
9. A charge transfer complex of an amino compound of claim 1 and m-dinitrobenzene.
10. A charge transfer complex of an amino compound of claim 1 and hexachlorocyclopentadiene.
11. A charge transfer complex of an amino compound of claim 1 and chlorofumaronitrile.
12. A charge transfer complex of an amino compound of claim 1 and p-tricyanovinyl-N,N-dimethylaniline.
13. The complex of claim 1 wherein the amino compound is tetrakis(N-pyrrolidinyl)ethylene.
14. The complex of claim 1 wherein the amino compound is tetrakis(N-piperidinyl)ethylene.
15. The complex of claim 1 wherein the amino compound is tetrakis(morpholino)ethylene.
16. The complex of claim 1 wherein the amino compound is tetrakis[N-(N'méthyl)piperazinyl]ethylene.
17. The complex of claim 1 wherein the amino compound is 1,1',3,3'-tetramethyl- $\Delta^{2,2'}$ -bi(imidazolidine).
18. The complex of claim 1 wherein the amino compound is 1,1',3,3'-tetraethyl- $\Delta^{2,2'}$ -bi(imidazolidine).
19. The complex of claim 1 wherein the amino compound is 1,3'-diethyl-1',3-dimethyl -  $\Delta^{2,2'}$  - bi(imidazolidine).
20. The complex of claim 1 wherein the amino compound is 1,1',3,3'-tetramethyl- $\Delta^{2,2'}$ -bi(hexahydropyrimidine).
21. A charge transfer complex of an amino compound of claim 1 and a quinone.
22. A charge transfer complex of tetrakis(dimethylamino)ethylene and a quinone.
23. A charge transfer complex of tetrakis(dimethylamino)ethylene and chloranil.
24. A charge transfer complex of tetrakis(dimethylamino)ethylene and bromanil.
25. A charge transfer complex of tetrakis(dimethylamino)ethylene and iodanil.
26. A charge transfer complex of tetrakis(dimethylamino)ethylene and tetrabromo-1,2-benzoquinone.
27. A charge transfer complex of tetrakis(dimethylamino)ethylene and diphenoquinone.
28. A charge transfer complex of tetrakis(dimethylamino)ethylene and tetracyanoethylene.
29. A charge transfer complex of tetrakis(dimethylamino)ethylene and m-dinitrobenzene.
30. A charge transfer complex of tetrakis(dimethylamino)ethylene and hexachlorocyclopentadiene.
31. A charge transfer complex of tetrakis(dimethylamino)ethylene and dichlorofumaronitrile.
32. A charge transfer complex of tetrakis(dimethylamino)ethylene and p-tricyanovinyl-N,N-dimethylaniline.
33. A charge transfer complex of tetrakis(N-pyrrolidinyl)ethylene and 7,7,8,8-tetracyanoquinodimethane.
34. A charge transfer complex of tetrakis(N-piperidino)ethylene and diphenoquinone.

No references cited.

WALTER A. MODANCE, Primary Examiner.  
IRVING MARCUS, L. D. ROSDOL, Examiners.